

Aug. 11, 1931.

J. L. DRAKE

1,818,204

## PROCESS AND APPARATUS FOR FORMING SHEET GLASS

Filed Jan. 20, 1928

2 Sheets-Sheet 1



Inventor  
*John L. Drake*

By Frank Fraser.

Attorney

Aug. 11, 1931.

J. L. DRAKE

1,818,204

PROCESS AND APPARATUS FOR FORMING SHEET GLASS

Filed Jan. 20, 1928

2 Sheets-Sheet 2



Inventor  
John L. Drake

Attorney

Frank Fraser

## UNITED STATES PATENT OFFICE

JOHN L. DRAKE, OF TOLEDO, OHIO, ASSIGNOR TO LIBBEY-OWENS-FORD GLASS COMPANY,  
OF TOLEDO, OHIO, A CORPORATION OF OHIO

## PROCESS AND APPARATUS FOR FORMING SHEET GLASS

Application filed January 20, 1928. Serial No. 248,028.

The present invention relates to a process and apparatus for forming sheet glass.

One of the objects of this invention is to provide a process and apparatus of this character whereby sheet glass may be expeditiously formed and sheets which are substantially flat and of predetermined dimensions obtained.

Another object of this invention is to provide a process and apparatus of this nature wherein molten glass is deposited upon a moving support and gradually reduced through successive stages to a sheet of substantially predetermined dimensions.

Still another object of this invention is to provide a process and apparatus of this nature wherein molten glass is first completely melted and refined in a receptacle and then deposited upon a moving surface and reduced to a sheet of substantially predetermined dimensions by spreading it outwardly from its center.

Still another object of this invention is to provide a process and apparatus of this nature wherein molten glass is first created in a receptacle and completely refined therein and then deposited upon a movable supporting surface moving in a substantially horizontal plane and rolled to sheet form by gradually reducing it in thickness while simultaneously increasing it in width.

Still another object of this invention is to provide such a process and apparatus wherein molten glass is deposited upon a temperature controlled moving support and gradually reduced while on said support through successive stages to a sheet of substantially predetermined dimensions.

Still another object of this invention is to provide a process and apparatus of this character wherein previously completely melted and refined molten glass is deposited upon a support moving in a horizontal plane and subjected to the action of co-operating rolling members whereby the molten glass is rolled through successive stages into a sheet of substantially predetermined dimensions.

Various other objects, advantages and novel details of construction of this invention will be made more apparent as this descrip-

tion proceeds, especially when considered in connection with the accompanying drawings, wherein:

Figure 1 is a fragmentary vertical longitudinal sectional view through a sheet forming apparatus constructed in accordance with this invention. 55

Figure 2 is a top plan view of the sheet forming mechanism illustrated in Figure 1.

Figures 3 to 6 inclusive are detail sectional views taken substantially on the planes indicated by lines 3-3, 4-4, 5-5, and 6-6 in Figure 1, and 60

Figure 7 is a fragmentary longitudinal sectional view through a modified construction of sheet forming mechanism. 65

Referring now to the drawings and more particularly to Figures 1 to 6 inclusive it will be noted that there is illustrated a movable support indicated generally by the reference character 10 and in the form of construction herein illustrated consisting essentially of a plurality of table sections or members 11 each of which is provided with rolls or wheels 12 by means of which these members may be moved and guided along a track or guideway 13. 70

Each table member 11 is provided with a substantially plane upper sheet supporting surface 14 and a continuous movable support is provided by employing a number of members 11 arranged end to end in abutting relation. Any desired form of coupling means such as indicated at 15 may be provided for detachably uniting the several table members so that a continuous unbroken surface is presented under the forming means yet to be referred to. In practice, the table members are moved along the trackways 13 end to end in abutting relation and 80 those table members which have moved under and passed the sheet forming mechanism are subsequently uncoupled from the train and again placed on the trackway 13 in advance of the sheet forming mechanism. 85 Furthermore, the table members 11 are of such a length and the depositing of the molten glass is so timed that a complete sheet is preferably formed on each table whereby the glass forming a single sheet does not 90 95 100

extend over the joint between two adjacent tables.

Co-operating with the movable support 10 are a plurality of rolls 16, 17, 18 and 19. These rolls are rotatably mounted by means of shafts 20 and while any preferred or desired means may be employed for rotating these rolls such means is herein illustrated as comprising gears or pinions 21 fixed to the shafts 20 and meshing with racks 22 arranged along the longitudinal edges of the table members 11. Thus as the table sections or movable supports move past the fixedly mounted rolls these rolls are rotated in timed relation with the movement of the movable support.

The rolls 16, 17 and 18 gradually taper from their centers toward their opposite ends while the roll 19 is cylindrical and co-operates with the movable support to form a straight sheet forming pass having straight parallel sides. The degree of taper of the several rolls 16, 17 and 18 gradually decreases from the first mentioned roll to the last mentioned one so that the rolls gradually approach cylindrical form.

The distance the roll 19 is spaced from the movable support 10 determines the thickness of the sheet produced. Each roll is also preferably provided at its opposite ends with collars or the like 23 which serve to prevent the molten glass from flowing beyond the ends of the rolls and each table section 11 of the movable support 10 is provided with longitudinally extending ledges 24 arranged adjacent the longitudinal edges thereof for co-operation with the collars 23 to define the limits within which the molten glass may flow laterally and to determine the width of the sheet.

By reason of the particular construction of the forming rolls the space between these rolls and the movable support varies, gradually decreasing from the roll 16 to the roll 19 so that the stream of molten glass passing therebetween is gradually reduced in thickness. Also because of the formation of these rolls the glass is spread outwardly from its center towards the opposite ends thereof and thus the stream while being gradually reduced in thickness is simultaneously increased in width so that the resultant sheet will be of substantially predetermined dimensions.

Means is provided for adequately controlling the temperature of the mass of molten glass as it is deposited upon the sheet forming means and of the sheet during the formative period. For this purpose a compartment or chamber 25 is provided through which the movable support passes, this chamber being provided with an opening 26 controlled by a suitable cover or gate 27. By removing the gate 27 a melting receptacle or pot 28 containing previously completely melted and refined molten glass

may be introduced into the compartment 25 and poured or deposited upon the movable support 10 to create the mass of molten glass 29.

The temperature of this compartment 25 may be controlled in any desired manner by any suitable heating means, and burners or other suitable heating means 30 can also be provided to control the temperature of the molten mass 29 prior to the time that it passes beneath the forming rolls to maintain the same in a plastic workable condition.

As the movable support passes out of compartment 25 it passes into compartment or chamber 31 in which the rolls 16, 17, 18 and 19 are located. The temperature of this compartment or chamber may also be controlled independently of the chamber 25 in any desired manner and burners or the like 32 are preferably employed to control the temperature of the glass as it passes under the rolls whereby to maintain the same in a plastic workable condition. The compartment 31 preferably extends to or adjacent to an annealing lehr 33 into which the formed sheet is conveyed by means of the movable support 10.

Means is also provided for controlling the temperature of each of the tables or supporting members 11. For this purpose each table is preferably of a hollow construction providing heat compartments or chambers 34 opening preferably as at 35 along the longitudinal sides thereof. Positioned along the path of travel of the table sections 11 are a plurality of burners 36, these burners being so positioned that the flames thereof play within or enter the heating compartments 34 through the openings 35 thereof. Thus as the movable table members 11 pass along the trackway 13 the interiors thereof are constantly subjected to the heat from the burners 36. In this manner the temperature of these tables may be adequately regulated or controlled. By reason of the foregoing it will be evident that the temperature of the glass may be adequately controlled from the time it is deposited in a molten mass until the sheet is completely formed.

While any desired or preferred means may be employed for moving the table members along the trackway 13 the means herein shown consists of a gear 37 engaging a rack 38 carried by the table members.

In Figure 7 a slightly modified form of construction is illustrated. In this form the mass of molten glass 39 is created in a melting pot or receptacle 40 and then deposited upon a movable support consisting of an endless belt 41 carried by pulleys or drums 42. Means 43 for maintaining the endless belt taut may and preferably is being provided.

The upper flight of the endless belt 41 is supported by means of a table or support 44 to prevent the same from sagging and

thus provides a rigid non-yieldable support upon which to deposit the mass of molten glass 39. Co-operating with the movable support is a plurality of rolls 45, 46, 47 and 48 similar in shape, construction and operation to the rolls 16, 17, 18 and 19 of the previously described construction. These rolls may be driven in any desired manner and co-operate with the support 44 in the manner previously described to gradually reduce the mass of molten glass through successive stages to a sheet of substantially predetermined dimensions. The formed sheet 50 is supported, upon leaving the endless belt 41, by means of a supporting member 51 and then passes between a pair of rolls 52 into an annealing lehr 53. The temperature of the supporting member 51 and of the rolls 52 may be controlled in any desired manner preferably by circulating a temperature control medium through their hollow interiors.

While several embodiments of the invention have been described and illustrated herein somewhat in detail it will be readily apparent to those skilled in this art that various changes, modifications and re-arrangements of the constructions illustrated may be resorted to without departing from the spirit and scope of the invention and to this end reservation is made to make such changes as may come within the purview of the accompanying claims.

Claims:

1. In the process of forming sheet glass, those steps which consist in depositing a mass of molten glass upon a movable support and moving said support to bring the molten glass under a plurality of forming rolls to subject the same to a series of successive rolling operations wherein the glass is reduced first at its center and the end portions then subsequently reduced gradually through successive stages to the same thickness to form a sheet of substantially predetermined thickness and width.

2. In the process of forming sheet glass, those steps which consist in depositing a mass of molten glass on a movable support within a temperature controlled chamber and gradually reducing the same while upon said support through successive stages to sheet form in a second temperature controlled chamber.

3. In sheet glass forming apparatus, a movable support for a mass of molten glass, a plurality of sheet forming rolls co-operating therewith to gradually reduce the molten glass through successive stages to sheet form and separate temperature controlled chambers enclosing said movable support at the point of deposit of said molten glass and said sheet forming rolls.

4. In sheet glass forming apparatus, a longitudinally moving support, means for depositing a mass of molten glass thereon, a

plurality of sheet forming rolls co-operating with said support to gradually reduce the molten glass through successive stages to sheet form, a chamber enclosing said movable support at the point of deposit of said molten glass, a second chamber in which said sheet forming rolls are located, and means for independently controlling the temperature of said chambers.

5. In sheet glass forming apparatus, a longitudinally moving supporting member, a plurality of temperature controlled chambers through which said support moves, means for depositing a mass of molten glass upon said support in one of said chambers a plurality of rolls located in another chamber and co-operating with said support to gradually reduce the mass of molten glass through successive stages to sheet form, and means for independently controlling the temperature of said chambers.

6. Sheet glass forming apparatus comprising in combination, a plurality of separate adjoining temperature controlled chambers, a continuous support movable through said chambers, means for controlling the temperature of said movable support, means for depositing a mass of molten glass upon said support within one of said chambers and sheet forming rolls located in another of said chambers and co-operating with said movable support to gradually reduce said molten glass through successive stages to a sheet of substantially predetermined thickness and width.

7. Sheet glass forming apparatus comprising in combination, a plurality of separate adjoining temperature controlled chambers, a continuous support movable through said chambers, means for controlling the temperature of said movable support, means for depositing a mass of molten glass upon said support within one of said chambers and a plurality of rolls arranged within another of said chambers and co-operating with said movable support to subject the mass of molten glass to successive rolling operations wherein the glass is spread outwardly from its center and gradually reduced through successive stages to a sheet of substantially predetermined thickness and width.

8. In the process of forming sheet glass, those steps which consist in depositing a mass of molten glass upon a moving support, gradually rolling the glass through successive stages to sheet form while upon said support, in then annealing the glass prior to removing it from said support, and in controlling the temperature of the glass contacting surface of said support during the formation of the sheet thereupon and its subsequent annealing.

9. In the process of forming sheet glass, those steps which consist in depositing a mass of molten glass upon a moving support, reducing the thickness of the glass while upon

said support first at its center, then gradually reducing the end portions through successive stages to the same thickness, and in then annealing the glass prior to removing it from said support.

5. 10. In the process of forming sheet glass, those steps which consist in depositing a mass of molten glass upon a moving support, reducing the thickness of the glass while upon said support first at its center, then gradually reducing the end portions through successive stages to the same thickness, then annealing the glass prior to removing it from said support, and in applying heat to the under-

10 15 said support first at its center, then gradually reducing the end portions through successive stages to the same thickness, then annealing the glass prior to removing it from said support, and in applying heat to the under-

15 20 said support during the formation of the sheet thereupon and its subsequent annealing.

11. In apparatus for forming sheet glass, a longitudinally moving, horizontal supporting member, means for depositing a mass of molten glass thereupon, and a plurality of forming rolls mounted above said support, said rolls being constructed to reduce the glass first at its center and to then gradually reduce the end portions through successive 25 30 stages to the same thickness whereby to form a sheet of substantially predetermined thickness.

12. In apparatus for forming sheet glass, a longitudinally moving, horizontal supporting member, means for depositing a mass of molten glass thereupon, and a plurality of forming rolls mounted above said supporting member and cooperating therewith to gradually reduce the glass through successive 35 40 stages to a sheet of substantially predetermined dimensions, the first roll adjacent the point of deposit of the molten glass upon the supporting member tapering from its center towards its opposite ends and the last roll furthest remote from said point being cylindrical.

13. In apparatus for forming sheet glass, a longitudinally moving, horizontal supporting member, means for depositing a mass of molten glass thereupon, a plurality of forming rolls mounted above said supporting member and cooperating therewith to gradually reduce the molten glass through successive 45 50 stages to sheet form, the first roll adjacent the point of deposit of the molten glass upon the supporting member tapering from its center towards its opposite ends and the succeeding following rolls progressively and gradually approaching cylindrical form.

14. In apparatus for forming sheet glass, a movable support adapted to receive a mass of molten glass thereupon, means cooperating with the support for reducing the glass to sheet form, said movable support being provided with heat chambers, and fixed means disposed in the course of travel of said support for heating said chambers as said support is moved past the same.

15. The process of forming sheet glass,

which consists in depositing a mass of molten glass upon a moving support, reducing the thickness of the glass while upon said support first at its center, and in then reducing the end portions to the same thickness.

16. The process of forming sheet glass, which consists in depositing a mass of molten glass upon a moving support, reducing the thickness of the glass while upon said support first at its center, and in then gradually reducing the end portions through successive 75 80 stages to the same thickness.

17. In apparatus for forming sheet glass, a movable support adapted to receive a mass of molten glass thereupon, means cooperating with the support for reducing the molten glass to sheet form, said movable support having internal heating chambers, and fixed means disposed at the opposite sides of the support in the course of travel thereof for directing heating flames into said chambers as said support is moved past the same.

Signed at Toledo, in the county of Lucas and State of Ohio, this 18th day of January 1928.

JOHN L. DRAKE.

70

75

80

85

90

95

100

105

110

115

120

125

130